

# United States Patent Office

2,924,544

Patented Feb. 9, 1960

1

2,924,544

## METALLURGICAL PROCESS FOR COLD-FINISHING STEEL

Elliot S. Nachtman, Park Forest, Ill., assignor to La Salle Steel Co., Hammond, Ind., a corporation of Delaware

No Drawing. Application October 22, 1956  
Serial No. 617,266

9 Claims. (Cl. 148—12)

This invention relates to a metallurgical process for use in the cold-finishing of steel bars, rods, tubing, wires, and other steel elements to improve mechanical and physical properties of the steel, and it relates more particularly to a new and improved process which is applicable to the cold finishing of steel to broaden mechanical and physical properties which can be developed in the steel, and to improve certain mechanical and physical properties for use of the steel in various and broadened applications.

This invention represents a modification and improvement over the inventions described in the copending applications of Nachtman and Moore, Serial No. 518,411, Serial No. 518,412, Serial No. 518,413, and Serial No. 518,414, filed June 27, 1955, now Patents No. 2,767,837, No. 2,767,835, No. 2,767,836 and No. 2,767,838, respectively.

It is an object of this invention to produce and to provide a method for producing steel products having improved mechanical and physical properties.

Another object of this invention is to provide a method which has application to the field of cold-finishing steels wherein the properties and characteristics of the steel are materially changed to increase the uniformity of properties and characteristics of steels of the same chemistry from heat to heat, to expand the range of physical and mechanical properties capable of being developed in the steel, to improve the values of physical and mechanical properties of the steel, and to produce steel products having new and improved characteristics and physical and mechanical properties of higher values.

In the aforementioned copending applications, the inventive concepts reside in the improvement in physical and mechanical properties of steel by the processing of the steel in an elevated-temperature-reduction step wherein the steel is advanced through a die to take a reduction in cross-sectional area while the steel is at a temperature within the range of 200° F. to the lower critical temperature (1100°—1200° F.) for the steel composition. Depending upon the temperature of the steel advanced through the die, various physical and mechanical properties of the steel can be markedly improved by comparison with the same steels which have been given the same reduction by advancement of the steel through the same die, but while the steel is at about room temperature. Thus, by controlling the temperature of the steel advanced through the die, by controlling the chemistry of the steel, and by controlling the amount of reduction that is taken, it has become possible, in an improved cold-finishing process, as the term is used in the trade, as distinguished from the finishing of steel while cold, to produce steel products having new and improved physical and mechanical properties and characteristics not avail-

able in steels fabricated by other means heretofore employed.

In a number of my copending applications filed concurrently herewith, description is made of further modifications and improvements in the elevated-temperature-reduction concept wherein; in one method, the steel is subjected to a cold reduction step in advance of the elevated-temperature reduction; in another method, the steel is normalized prior to advancement through a die to effect reduction in cross-sectional area while the steel is at an elevated temperature within the range described; and, in a third modification, the steel is subjected to a heat-treating step to anneal the steel prior to advancement of the steel through a die to effect reduction in cross-sectional area while the steel is at a temperature and range of 200° F. to the lower critical temperature for the steel composition. In each of these processes described, utilization continues to be made of the characteristics of the steel relating to strain-hardening and to hardening by some mode of precipitation when worked at elevated temperature, similar to age-hardening, to produce steels having improved physical and mechanical properties. The heat treatments or the cold reduction step taken in advance of the elevated-temperature-reduction step provides for no phase change of the steel but changes are made in values and in the range of values capable of being developed by the combination of the described steps.

The concepts of this invention reside in the method of processing steel in an operation applicable to the cold-finishing of steel to cause new and improved physical and mechanical properties to be developed in the steel by the combination of the phenomena made available by taking a reduction at elevated temperature, as described in the aforementioned copending applications, but in which the steel has been treated to effect a phase change in the steel prior to the elevated-temperature-reduction step. In accordance with the practice of this invention, the steel is processed by a combination of steps which includes heating the steel to austenitizing temperature and rapidly cooling the steel from austenitizing temperature to about ambient temperature to produce a phase change in the steel, tempering the steel by heat treatment to a desired temperature below the lower critical temperature of the steel composition, and then subsequently working the steel in an elevated temperature reduction step, as, for example, by advancing the steel through a die to effect reduction in cross-sectional area while the steel is at a temperature within the range of 200° F. to the lower critical temperature for the steel composition, such, for example, as at a temperature within the range of 200° F. to 1100°—1200° F. The combination of steps described, which combines the phenomena of strain-hardening and age-hardening with a phase change in the steel, produces a steel having considerably different combinations of physical and mechanical properties and characteristics. The physical and mechanical properties developed in the steel differ in many respects from the properties made available in steels by a cold reduction or by reduction at elevated temperature without a phase change having previously been effected in the steel.

The process of austenitizing, rapidly cooling the steel from austenitizing temperature to about room temperature, as by quenching the steel in oil or water, tempering the quenched steel, and subsequently reducing the quenched and tempered steel at an elevated temperature results in a simple and efficient method, capable of use

in the cold-finishing of steel, to provide a wide range of physical and mechanical properties not heretofore available in steels of corresponding chemistry. Some of the more significant improvements secured in steels processed in the manner described reside in the higher elasticity and impact-strength properties produced in the steel at equivalent strength levels by comparison with steels processed by conventional methods or by methods of the type described in the aforementioned copending applications.

Included among the physical and mechanical properties influenced by processing steels in the manner described are the strength properties of the steel including tensile strength, impact strength, flexure strength and the like, and other properties such as elasticity, elongation, hardness, surface roughness, machinability, proportional limits and the like. As described in the aforementioned copending applications, the properties of machinability, tensile strength, flexure strength, yield strength, proportional limits, impact strength, and hardness are usually beneficially affected when the steel is advanced through a die to take a reduction in cross section while the steel is at an elevated temperature in the range of 200° F. to the lower critical temperature of the steel composition and preferably while the steel is at a temperature within the range of 450° to 850° F.

These same phenomena of improvements in physical and mechanical properties of steel by reduction at elevated temperature are capable of full development in steels in which the described phase change has been effected by austenitizing, quenching to about room temperature, and tempering, except that a broader range of properties are capable of being developed with greater uniformity of properties from heat to heat. Material and significant improvements are available in the elasticity and impact-strengths of the steels at comparable strength levels, and the elevated-temperature-reduction step, capable of being taken while the steel is at a temperature of 200° F. to the lower critical temperature for the steel, is broadened in a preferred range to include temperatures within the range of 200° to 900° F.

The characteristics described are capable of development with hot-rolled steels of the type which are cold-finished by the processes of drawing or extrusion, for example. Steels which may be used in the practice of this invention are of the type which strain-harden or harden by some mode of precipitation when worked at an elevated temperature. Representative are the plain carbon, low carbon, or high carbon and low-alloy steels of the easy-to-draw type which, in the hot-rolled state, include the non-austenitic steels having a pearlitic structure in a matrix of free ferrite. These are to be distinguished from the hard-to-draw, high-speed, or carbon-tool steels, and the high-alloy steels and stainless steels. In the process of austenitizing and quenching, the structure of the steel is believed to be converted to a steel which contains either bainite or martensite, alone or in combination. The quenched steel is hard to draw at room temperature, but can be drawn or otherwise reduced in cross-section when advanced through the die when the steel is at a temperature within the range described for the elevated-temperature-reduction step of from 200° F. to the lower critical temperature of 1100°-1200° F. for the steel composition, and preferably at a temperature within the range of 200°-900° F.

In the process described, temperature and temper have an influence on the characteristics that are developed in the steel and by proper selection of the temperature at which the steel is tempered, the temperature of the steel advanced through the die in the elevated-temperature-reduction step, the amount of reduction that is taken and the chemistry of the steel, it is possible to produce steel products of widely varying physical and mechanical properties, and stress characteristics to produce steel products having new and improved combinations of properties. Treatment of the steel after the elevated-tempera-

ture-reduction step, as by slow cooling in air or by rapidly cooling, as by quenching in oil or water, bears very little material effect upon the properties developed in the steel except that rapid cooling tends to produce steels having lower levels of stress, and tends to produce steels having compressive stresses in the surface portions to provide steel products characterized by less warpage. These characteristics will become evident from the data which will hereinafter be set forth, representing the practice of this invention.

As used herein, the term "elevated-temperature-reduction" is meant to include the process of cold-finishing steel wherein the steel is advanced to a draw die to effect reduction in cross-sectional area while the steel is at an elevated temperature within the range of 200° F. to the lower critical temperature, and preferably at a temperature of 200°-900° F. Included also, is the process of extruding by advancement of the steel through an extruding die or by advancement of the steel through a roller die for reduction in cross-sectional area while the steel is at the desired elevated temperature. While not equivalent from the standpoint of the process, many of the characteristics described are also capable of development in other processes for working steel to effect reduction in cross-sectional area, such as by the process of rolling steels to effect reduction in cross-sectional area while the steel is at an elevated temperature within the range described.

The phrase "austenitizing" and quenching is meant to embody the usual meaning of the term as employed in the steel trade. It includes the step of heating the steel to austenitizing temperature for the steel composition, usually within the range of 1500°-1600° F., followed by rapidly cooling the steel to room temperature, as by means of an oil quench or water quench, to freeze the phase change in the steel whereby a steel believed to contain bainite or martensite, or combinations thereof, is produced. The austenitized steel is then tempered by heating the steel to a temperature below the lower critical temperature, and preferably at a temperature within the range of 200°-1200° F., and preferably, the tempering operation is carried out by heating the austenitized and quenched steel to a temperature within the range of 400°-900° F. The tempered steel may be cooled down to room temperature and subsequently re-heated to the desired temperature for the elevated-temperature-reduction step, or it may be adjusted directly from the tempering temperature to the temperature for elevated-temperature-reduction.

The following will illustrate the practice of this invention, including the effect of tempering the steel at various temperatures within the range of 200° to 1100° F., and the effect of temperature on the properties developed in the steel when the austenitized, quenched, and tempered steels are advanced through the die to effect reduction in cross-sectional area while the steel is at an elevated temperature within the range described.

The concepts of this invention will hereinafter be illustrated by reference to the processing of four steels which are taken as representative of the classes of steels which may be employed. These representative steels will hereinafter be referred to as C-1018, C-1144, C-1080, and 4140. The following is a ladle analysis of these steels in which the major ingredients, other than iron, are set forth:

| Grade  | Chemistry |      |      |      |     |       |       |
|--------|-----------|------|------|------|-----|-------|-------|
|        | C         | Mn   | P    | S    | Si  | Cr    | Mo    |
| C-1018 | .18       | .88  | .015 | .037 | .06 | ----- | ----- |
| C-1144 | .45       | 1.51 | .018 | .28  | .22 | ----- | ----- |
| C-1080 | .86       | .79  | .010 | .031 | .20 | ----- | ----- |
| 4140   | .43       | .88  | .018 | .020 | .26 | .86   | .18   |

The procedures for processing the steels and the conditions for testing the steels in the development of the data set forth in the following tables will hereinafter briefly be described, along with some of the terms which are employed, as used in the specification and claims.

#### PROCEDURE

The hot-rolled steel bars, as received, are de-scaled by pickling in sulphuric acid and limed to prevent rusting. Lime has the advantage of preventing formation of a tight scale in a normal furnace atmosphere at elevated temperature.

All of the hot-rolled, pickled and limed bar stock to be processed in accordance with the teaching of this invention, was heated to the austenitizing temperature by means of a Hevi Duty electric furnace. It will be understood that other means for heating the steels to austenitizing temperature may be employed in the practice of this invention. For austenitizing, the steels were heated to the following temperature:

|        |      |
|--------|------|
| C-1018 | 1600 |
| C-1144 | 1500 |
| C-1080 | 1500 |
| 4140   | 1550 |

For quenching the steels heated to austenitizing temperature, the steels were immersed in an oil bath. It will be understood that other means for rapidly cooling the austenitized steel to ambient temperature may be employed, and that such other means are well known to the trade.

For tempering, the austenitized and quenched steels were re-heated in suitable heat-treating furnaces. The steels were re-heated for tempering to a temperature within a range of 200°-1100° F., as indicated by the data set forth in the following tables.

The austenitized, quenched, and tempered steel bars can be cooled down from the temperature of tempering to the temperature desired for advancement through the die in the elevated-temperature-reduction step. In the data developed, as representative of the practice of this invention, the tempered steel was cooled back down to about ambient temperature and then re-heated from ambient temperature, as in a gas-fired furnace, to temperatures desired for taking the elevated temperature reduction step. The steel bars were lubricated in advance of drawing with a suitable drawing compound. In the drawing step, the steels were advanced through a die having the characteristics of the die contour described in the copending application of Kyle, Nachtman, Landis and Kelly, Serial No. 484,726, filed January 28, 1955.

#### DEFINITIONS

"Percent reduction" is meant to relate to the true reduction, as represented by the formula

$$\frac{D_1 - D_2}{D_1} \times 100 = \text{percent reduction}$$

wherein  $D_1$  is the original hot-rolled diameter of the steel and  $D_2$  is the final diameter of the steel. The original diameters of the steels are as follows:

|        |               |
|--------|---------------|
| C-1018 | 3/4" round    |
| C-1144 | 5/8" round    |
| C-1080 | 9/16" round   |
| 4140   | 1 1/16" round |

"Proportional limits" is intended to correspond to the point in the stress-strain curve where the greatest stress that the material is capable of sustaining without deviation from the law of proportionality of stress to strain occurs (Hooke's law).

Warpage factor is directly related to residual stress. The warpage value is an indication of the concentration and character of the longitudinal stresses present in steel. The residual stress is obtained by means of a warpage test wherein the length of the test piece is determined as being five times the diameter plus two inches. The test pieces are slotted through a diameter for a distance five times the diameter of the piece. The length of the slot is recorded and the maximum diameter perpendicular to the slot is also recorded. The differences between the diameter before slotting and after slotting represents the flare caused by the presence of residual stresses. The flare is considered positive, indicative of a preponderance of tensile stresses in the steel, if the bar expands upon slotting. The flare is considered negative, indicative of preponderance of compressive stresses in the steel, if the ends move toward the cut made through the diameter. The warpage values determined for evaluation are calculated on the following equation:

$$\text{Warpage factor} = \frac{(D_0)(D_F)}{(L_S)^2} \times 100$$

where

$D_0$ =the original diameter of the bar before cutting the slot

$D_F$ =the diameter differential before and after cutting the slot (flare)

$L_S$ =length of slot

Izod impact represents the impact in foot-pounds obtained by averaging the impact results from three equidistant forty-five degree notches (0.13" deep) at 70° F. on a 0.45" diameter round x 4 1/2" long specimen.

Hardness, represented by a diamond pyramid number (D.P.N.) was measured on a Gries reflex-testing machine employing 136 pyramid diamond at a 50 kilogram (kg.) load.

The term "elevated-temperature drawing" (ETD) is meant to define the taking of a reduction in the cross-section of the steel by advancement of the steel through a die while at a temperature within the range of 200° F. to the lower critical temperature for the steel composition (1100°-1200° F.).

Table I

[C-1018 Steel: Austenitized by heating to 1600° F. Quenched in oil. Tempered at 400° F. Drawn to 17.2% reduction. Cooled in air after drawing.]

| Temp. of Draw, ° F.                                | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, D.P.N., MR |
|----------------------------------------------------|--------------------------|------------------------|---------------------------|-----------------------|----------------|-------------------------------|----------------------|
| Hot Roll <sup>1</sup>                              | 68,375                   | 46,875                 | 36.0                      | 67.9                  | + .021         | 87.0                          | 151                  |
| As Quenched <sup>1</sup>                           | 164,000                  | 109,000                | 11.5                      | 22.6                  | - .400         | 17.0                          | 371                  |
| H.R. Quenched <sup>1</sup> and Tempered at 400° F. | 109,750                  | 75,000                 | 19.5                      | 55.6                  | - .240         | 43.0                          | 285                  |
| 280                                                | 138,000                  | 137,500                | 9.5                       | 42.8                  | + .040         | 8.7                           | 343                  |
| 400                                                | 123,000                  | 123,000                | 14.5                      | 62.0                  | - .110         | <sup>2</sup> (47.3)           | 296                  |
| 685                                                | 147,500                  | 147,500                | 9.0                       | 46.1                  | + .052         | 8.7                           | 356                  |
| 900                                                | 97,000                   | 87,000                 | 17.5                      | 68.3                  | + .023         | <sup>2</sup> (61.3)           | 226                  |

<sup>1</sup> Not drawn.

<sup>2</sup> Averaged values for a fibrous fracture—not a clean break test.

Table II

[C-1018 Steel: Austenitized by heating to 1600° F. Quenched in oil. Tempered at 400° F. Drawn to 17.2% reduction. Quenched in water after drawing.]

| Temp. of Draw, ° F.                                | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|----------------------------------------------------|--------------------------|------------------------|---------------------------|-----------------------|----------------|-------------------------------|-------------------|
| Hot Roll <sup>1</sup>                              | 68,375                   | 46,875                 | 36.0                      | 67.9                  | +.021          | 87.0                          | 151               |
| As Quenched <sup>1</sup>                           | 164,000                  | 109,500                | 11.5                      | 22.6                  | -.400          | 17.0                          | 371               |
| H.R. Quenched <sup>1</sup> and Tempered at 400° F. | 109,750                  | 75,000                 | 19.5                      | 55.6                  | -.240          | 43.0                          | 285               |
| 230                                                | 138,000                  | 137,500                | 9.5                       | 42.8                  | +.040          | 8.7                           | 343               |
| 405                                                | 134,250                  | 134,250                | 11.0                      | 48.9                  | -.127          | 22.3                          | 280               |
| 570                                                | 152,000                  | 152,000                | 9.0                       | 38.4                  | +.081          | 6.3                           | 356               |
| 900                                                | 99,000                   | 88,750                 | 23.0                      | 67.9                  | -.133          | <sup>2</sup> (54.3)           | 234               |

<sup>1</sup> Not drawn.

<sup>2</sup> Averaged value for a fibrous fracture—not a clean break test.

Table III

[C-1018 Steel: Austenitized by heating to 1600° F. Quenched to room temperature in oil. Tempered at 900° F. Drawn to 17.2% reduction. Cooled in air after drawing.]

| Temp. of Draw, ° F.                                | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|----------------------------------------------------|--------------------------|------------------------|---------------------------|-----------------------|----------------|-------------------------------|-------------------|
| Hot Roll <sup>1</sup>                              | 68,375                   | 46,875                 | 36.0                      | 67.9                  | +.021          | 87.0                          | 151               |
| Hot Roll <sup>1</sup> As quenched                  | 164,000                  | 109,500                | 11.5                      | 22.6                  | -.400          | 17.0                          | 371               |
| H.R. Quenched <sup>1</sup> and Tempered at 900° F. | 90,750                   | 72,000                 | 25.5                      | 31.7                  | -.069          | <sup>2</sup> (72.7)           | 213               |
| 200                                                | 117,750                  | 117,500                | 11.5                      | 60.7                  | -.058          | <sup>2</sup> (46.0)           | 262               |
| 380                                                | 127,000                  | 127,000                | 13.0                      | 49.7                  | +.190          | 25.0                          | 291               |
| 580                                                | 128,750                  | 128,750                | 13.0                      | 55.9                  | +.029          | 19.0                          | 303               |
| 900                                                | 101,750                  | 92,000                 | 24.0                      | 69.2                  | 0              | <sup>2</sup> (74.7)           | 241               |

<sup>1</sup> Not drawn.

<sup>2</sup> Averaged values for a fibrous fracture—not a clean break test.

Table IV

[C-1144 Steel: Austenitized by heating to 1500° F. Quenched to room temperature in oil. Tempered at 1100° F. Drawn to take a 21.6% reduction. Air-cooled after drawing.]

| Temp. of Draw, ° F.                                  | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|------------------------------------------------------|--------------------------|------------------------|---------------------------|-----------------------|----------------|-------------------------------|-------------------|
| Hot Roll <sup>1</sup>                                | 108,000                  | 70,500                 | 23.0                      | 46.1                  | +.004          | 32.7                          | 220               |
| Hot Roll <sup>1</sup> as Quenched                    | 290,000                  | 236,500                | 6.0                       | 20.0                  | +.137          | 4.3                           | 492               |
| H.R. Quenched <sup>1</sup> and Tempered at 1,100° F. | 126,250                  | 115,500                | 20.0                      | 54.4                  | +.046          | 35.7                          | 285               |
| 205                                                  | 145,250                  | 125,500                | 10.0                      | 36.2                  | +.888          | 35.3                          | 291               |
| 400                                                  | 144,750                  | 133,750                | 12.5                      | 47.3                  | +.789          | 36.7                          | 301               |
| 430                                                  | 151,500                  | 142,000                | 11.5                      | 46.5                  | +.810          | 37.7                          | 301               |
| 515                                                  | 151,750                  | 149,500                | 9.0                       | 45.3                  | +.810          | 30.7                          | 312               |
| 600                                                  | 162,500                  | 162,500                | 9.0                       | 39.7                  | +.803          | 25.7                          | 336               |
| 630                                                  | 162,750                  | 162,750                | 9.5                       | 40.6                  | +.661          | 29.0                          | 336               |
| 745                                                  | 144,500                  | 142,500                | 16.0                      | 48.1                  | +.121          | 41.0                          | 318               |
| 830                                                  | 137,500                  | 133,500                | 18.0                      | 48.7                  | +.057          | 42.3                          | 301               |
| 965                                                  | 125,750                  | 117,500                | 22.0                      | 54.4                  | +.043          | 52.7                          | 271               |

<sup>1</sup> Not drawn.

Table V

[C-1144 Steel: Austenitized by heating to 1500° F. Quenched in oil. Tempered at 900° F. Drawn to take 21.6% reduction. Air-cooled after drawing.]

| Temp. of Draw, ° F.                                    | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|--------------------------------------------------------|--------------------------|------------------------|---------------------------|-----------------------|----------------|-------------------------------|-------------------|
| Hot Roll <sup>1</sup>                                  | 108,000                  | 70,500                 | 23.0                      | 46.1                  | +.004          | 32.7                          | 220               |
| Hot Roll <sup>1</sup> as Quenched                      | 290,000                  | 236,500                | 6.0                       | 20.0                  | +.137          | 4.3                           | 492               |
| Hot Roll <sup>1</sup> Quenched and Tempered at 900° F. | 166,500                  | 156,000                | 14.5                      | 46.5                  | +.014          | 25.0                          | 371               |
| 250                                                    | 181,750                  | 180,000                | 11.5                      | 42.3                  | +.125          | 51.5                          | 350               |
| 350                                                    | 198,750                  | 193,000                | 11.0                      | 41.5                  | +.123          | 50.0                          | 371               |
| 460                                                    | 199,500                  | 198,000                | 9.0                       | 33.0                  | +.081          | 41.0                          | 386               |
| 610                                                    | 213,750                  | 212,500                | 8.0                       | 35.3                  | +.107          | 42.0                          | 402               |
| 715                                                    | 195,000                  | 193,000                | 12.5                      | 41.0                  | +.576          | 32.5                          | 402               |
| 740                                                    | 187,000                  | 184,500                | 11.5                      | 45.3                  | +.576          | 36.0                          | 394               |
| 815                                                    | 174,000                  | 168,000                | 16.0                      | 47.3                  | +.320          | 41.0                          | 371               |
| 860                                                    | 167,000                  | 160,000                | 16.0                      | 44.9                  | +.199          | 24.0                          | 364               |
| 880                                                    | 160,000                  | 153,750                | 15.0                      | 43.2                  | +.142          | 27.0                          | 350               |

<sup>1</sup> Not drawn.

Table VI

[C-1144 Steel: Austenitized by heating to 1500° F. Quenched in oil. Tempered at 600° F. Drawn to take 21.6% reduction. Air-cooled after drawing.]

| Temp. of Draw, ° F.                                | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|----------------------------------------------------|--------------------------|------------------------|---------------------------|-----------------------|----------------|-------------------------------|-------------------|
| Hot Roll <sup>1</sup>                              | 108,000                  | 70,500                 | 23.0                      | 46.1                  | +.004          | 32.7                          | 220               |
| Hot Roll <sup>1</sup> as Quenched                  | 290,000                  | 236,500                | 6.0                       | 20.0                  | +.137          | 4.3                           | 324               |
| H.R. Quenched <sup>1</sup> and Tempered at 600° F. | 245,000                  | 216,000                | 9.0                       | 28.9                  | +.044          | 2.7                           | 318               |
| 275 <sup>2</sup>                                   |                          |                        |                           |                       | +2.550         |                               | 378               |
| 300 <sup>2</sup>                                   |                          |                        |                           |                       | +1.532         |                               | 420               |
| 530                                                | 222,000                  |                        | 0                         | 0                     | +1.552         | 9.3                           | 511               |
| 600                                                | 270,000                  | 268,000                | 0.7                       | 2.2                   | +1.329         | 9.0                           | 526               |
| 635                                                | 247,000                  | 243,000                | 4.3                       | 14.5                  | +1.075         | 8.7                           | 490               |
| 650                                                | 220,000                  | 211,000                | 9.7                       | 34.5                  | +.651          | 15.0                          | 438               |
| 750                                                | 176,000                  | 172,500                | 11.0                      | 46.1                  | +.085          | 25.0                          | 370               |
| 820                                                | 154,500                  | 150,500                | 13.0                      | 47.7                  | +.064          | 37.6                          | 330               |
| 1,000                                              | 135,000                  | 128,500                | 15.0                      | 50.1                  | +.035          | 52.0                          | 296               |

<sup>1</sup> Not drawn.<sup>2</sup> [Bars split in half when cut on the abrasive saw about 24 hours after drawing cycle.]

Table VII

[C-1144 Steel: Austenitized by heating to 1500° F. Quenched in oil. Tempered at 400° F. Drawn to take 21.6% reduction. Air-cooled after drawing.]

| Temp. of Draw, ° F.                                | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|----------------------------------------------------|--------------------------|------------------------|---------------------------|-----------------------|----------------|-------------------------------|-------------------|
| Hot Roll <sup>1</sup>                              | 108,000                  | 70,500                 | 23.0                      | 46.1                  | +.004          | 32.7                          | 220               |
| Hot Roll <sup>1</sup> as Quenched                  | 290,000                  | 236,500                | 6.0                       | 20.0                  | +.137          | 4.3                           | 324               |
| H.R. Quenched <sup>1</sup> and Tempered at 400° F. | 297,500                  | 175,500                | 7.9                       | 22.2                  | +.093          | 4.0                           | 330               |
| 520 <sup>2</sup>                                   |                          |                        |                           |                       |                |                               |                   |
| 580                                                | 347,000                  | 341,500                | 4.3                       | 16.0                  | +1.718         |                               | 610               |
| 660                                                | 272,000                  | 269,000                | 6.0                       | 31.7                  | +.818          | 7.3                           | 526               |
| 720                                                | 214,000                  | 212,500                | 11.0                      | 43.6                  | +.505          | 37.0                          | 438               |
| 760                                                | 207,250                  | 204,000                | 13.0                      | 42.3                  | +.484          | 27.7                          | 429               |
| 825                                                | 178,000                  | 170,500                | 14.5                      | 45.3                  | +.299          | 25.0                          | 386               |
| 890                                                | 162,750                  | 154,500                | 17.5                      | 47.7                  | +.135          | 31.3                          | 343               |

<sup>1</sup> Not drawn.<sup>2</sup> [Short specimen—Bar broke upon drawing.]

Table VIII

[C-1080 Steel: Austenitized at 1500° F. Tempered at 1200° F. Drawn to take 15.7% reduction. Air-cooled after drawing.]

| Temp. of Draw, ° F.                                  | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|------------------------------------------------------|--------------------------|------------------------|---------------------------|-----------------------|----------------|-------------------------------|-------------------|
| Hot Roll <sup>1</sup>                                | 144,500                  | 76,000                 | 12.5                      | 17.0                  | +.025          | 4.7                           | 296               |
| Hot Roll <sup>1</sup> as Quenched                    | 204,000                  |                        |                           |                       | -.061          | 2.0                           | 436               |
| H.R. Quenched <sup>1</sup> and Tempered at 1,200° F. |                          |                        |                           |                       |                |                               |                   |
| 133,500                                              | 103,000                  |                        | 21.0                      | 41.9                  | -.002          | 34.7                          | 276               |
| 154,250                                              | 133,000                  |                        | 12.5                      | 43.2                  | +.039          | 20.0                          | 324               |
| 152,000                                              | 128,000                  |                        | 13.0                      | 38.4                  | +.140          | 22.0                          | 301               |
| 152,250                                              | 138,750                  |                        | 12.5                      | 41.9                  | +.101          | 21.7                          | 312               |
| 158,500                                              | 153,000                  |                        | 9.0                       | 41.5                  | +.070          | 16.0                          | 324               |
| 169,500                                              | 169,500                  |                        | 7.0                       | 36.2                  | +.031          | 13.0                          | 312               |
| 170,250                                              | 170,000                  |                        | 9.0                       | 40.2                  | -.008          | 12.7                          | 318               |
| 152,750                                              | 142,000                  |                        | 14.0                      | 34.8                  | +.070          | 22.0                          | 307               |
| 142,000                                              | 124,500                  |                        | 16.5                      | 40.6                  | +.054          | 31.7                          | 296               |
| 132,500                                              | 107,500                  |                        | 20.0                      | 38.9                  | +.023          | 38.7                          | 285               |

<sup>1</sup> Not drawn.<sup>2</sup> Estimated from averaged hardness values of quenched specimens—Material appears to be very brittle and difficult to machine in the "as quenched" condition.

Table IX

[C-1080 Steel: Austenitized at 1500° F. Tempered at 700° F. Drawn to take 15.7% reduction. Air-cooled after drawing.]

| Temp. of Draw, ° F.                                | Tensile Strength, p.s.i. | Yield Strength, p.s.i. | Elongation, 1/4", Percent | Red. of Area, Percent | Warpage Factor | Izod Impact, 70° F., Ft.-Lbs. | Hardness, DPN, MR |
|----------------------------------------------------|--------------------------|------------------------|---------------------------|-----------------------|----------------|-------------------------------|-------------------|
| Hot Roll <sup>1</sup>                              | 144,500                  | 76,000                 | 12.5                      | 17.0                  | +.025          | 4.7                           | 296               |
| Hot Roll <sup>1</sup> as Quenched                  | 204,000                  |                        |                           |                       | -.061          | 2.0                           | 436               |
| H.R. Quenched <sup>1</sup> and Tempered at 700° F. |                          |                        |                           |                       |                |                               |                   |
| 256,000                                            | 217,500                  |                        | 10.0                      | 25.1                  | +.093          | 5.3                           | 490               |
| 261,000                                            |                          |                        | 0                         | 0                     | +.140          | 4.0                           | 502               |
| 270,000                                            |                          |                        | 0                         | 0                     | .318           | 4.0                           | 448               |
| 287,000                                            |                          |                        | 0                         | 0                     | .210           | 4.0                           | 429               |
| 303,000                                            | 303,000                  |                        | 3.6                       | 14.1                  | +.140          | 5.3                           | 438               |
| 620                                                | 288,000                  | 280,500                | 6.4                       | 21.6                  | +.194          | 5.6                           | 479               |
| 680                                                | 251,000                  | 238,500                | 8.6                       | 30.3                  | +.124          | 9.0                           | 458               |
| 765                                                | 209,250                  | 191,250                | 11.5                      | 32.1                  | +.078          | 12.0                          | 420               |
| 840                                                | 182,500                  | 157,500                | 13.0                      | 26.5                  | +.047          | 16.3                          | 358               |
| 900                                                | 156,000                  | 134,750                | 14.5                      | 29.3                  | +.016          | 25.3                          | 318               |

<sup>1</sup> Not drawn.<sup>2</sup> Estimated from averaged hardness values of quenched specimens—material appears to be very brittle and difficult to machine in the "as quenched" condition.

Table X

[4140 Steel: Austenitized at 1550° F. Tempered at 1100° F. Drawn to take 19.9% reduction. Air-cooled after drawing.]

| Temp. of Draw, ° F.                                  | Tensile Strength, p.s.i. | Yield Strength, p.s.i. | Elongation, 1.4", Percent | Red. of Area, Percent | Warpage Factor | Izod Impact, 70° F., Ft.-Lbs. | Hardness, DPN, MR |
|------------------------------------------------------|--------------------------|------------------------|---------------------------|-----------------------|----------------|-------------------------------|-------------------|
| Hot Roll <sup>1</sup>                                | 140,000                  | 105,750                | 15.0                      | 42.8                  | -.004          | 9.0                           | 307               |
| Hot Roll <sup>1</sup> as Quenched                    | 286,000                  | 231,000                | 12.1                      | 42.8                  | +.409          | 25.7                          | 448               |
| H.R. Quenched <sup>1</sup> and Tempered at 1,100° F. | 159,000                  | 149,750                | 17.5                      | 62.0                  | -.018          | 52.0                          | 356               |
| 250                                                  | 181,000                  | 173,750                | 13.0                      | 55.6                  | +.077          | <sup>2</sup> (46.3)           | 350               |
| 425                                                  | 177,000                  | 172,000                | 12.5                      | 52.5                  | +.121          | <sup>2</sup> (47.0)           | 356               |
| 505                                                  | 179,750                  | 179,500                | 14.5                      | 56.3                  | +.083          | <sup>2</sup> (42.0)           | 371               |
| 590                                                  | 190,500                  | 190,000                | 12.5                      | 55.2                  | +.115          | <sup>2</sup> (48.0)           | 378               |
| 690                                                  | 189,500                  | 189,500                | 13.0                      | 53.2                  | +.147          | <sup>2</sup> (37.0)           | 386               |
| 805                                                  | 178,250                  | 177,500                | 17.5                      | 55.9                  | +.281          | <sup>2</sup> (45.0)           | 386               |
| 900                                                  | 171,250                  | 168,000                | 17.5                      | 50.9                  | +.077          | 50.5                          | 371               |
| 960                                                  | 158,250                  | 153,750                | 21.0                      | 59.5                  | +.121          | <sup>2</sup> (63.0)           | 343               |

<sup>1</sup> Not drawn.

<sup>2</sup> Averaged values for fibrous fracture—not a clean break test.

Table XI

[4140 Steel: Austenitized at 1550° F. Tempered at 600° F. Drawn to take 19.9% reduction. Air-cooled after drawing.]

| Temp. of Draw, ° F.                                | Tensile Strength, p.s.i. | Yield Strength, p.s.i. | Elongation, 1.4", Percent | Red. of Area, Percent | Warpage Factor | Izod Impact, 70° F., Ft.-Lbs. | Hardness, DPN, MR |
|----------------------------------------------------|--------------------------|------------------------|---------------------------|-----------------------|----------------|-------------------------------|-------------------|
| Hot Roll <sup>1</sup>                              | 140,000                  | 105,750                | 15.0                      | 42.8                  | -.004          | 9.0                           | 307               |
| Hot Roll <sup>1</sup> as Quenched                  | 286,000                  | 231,000                | 12.1                      | 42.8                  | +.409          | 25.7                          | 448               |
| H.R. Quenched <sup>1</sup> and Tempered at 600° F. | 262,000                  | 225,000                | 13.0                      | 49.7                  | +.077          | 12.7                          | 539               |
| 500                                                | 279,000                  | -----                  | 0                         | 0                     | +.396          | 7.3                           | 594               |
| 615                                                | 275,000                  | -----                  | 0                         | 0                     | +.491          | 10.7                          | 565               |
| 720                                                | 261,000                  | 247,500                | 9.3                       | 41.0                  | +.617          | 16.7                          | 513               |
| 815                                                | 206,500                  | 206,500                | 14.5                      | 44.9                  | +.287          | 33.0                          | 429               |
| 910                                                | 179,750                  | 179,500                | 19.0                      | 58.1                  | +.064          | <sup>2</sup> (53.7)           | 386               |
| 980                                                | 154,000                  | 153,000                | 22.5                      | 62.0                  | +.013          | <sup>2</sup> (51.3)           | 330               |

<sup>1</sup> Not drawn.

<sup>2</sup> Averaged values for fibrous fracture—not a clean break test.

It will be apparent from the foregoing that the parabolic curve characteristic of the strength properties developed by elevated temperature reduction (ETD) without austenitizing, quenching and tempering is also capable of development in steels processes in accordance with the practice of this invention; that is, the steels which are austenitized, quenched, tempered and reduced at elevated temperatures. The range of properties of the austenitized, quenched, tempered and elevated drawn steels differs, however, from those developed by elevated temperatures alone and, in addition, improvements are secured in elasticity and machinability as will hereinafter be illustrated.

The foregoing tables clearly illustrate the improvements in tensile strength, yield strength and hardness in steels processed in accordance with the teachings of this invention over correspondingly austenitized, quenched and tempered steels drawn to effect an equivalent reduction at ambient temperature. The same improvements are generally made available whether the drawn steel is air-cooled or quenched after drawing. Ductility, as measured by percent elongation and reduction of area, is improved by elevated temperature reduction over cold drawing for the austenitized, quenched, and tempered steels for both air-cooled and quenched steels. Residual stress as measured by warpage stress is improved also but mostly in high-tempered quenched steels, such, for example, as the C1018 steel. Izod impact is improved in both air-cooled and quenched steels which have been tempered after austenitizing.

The data hereinafter set forth compares the properties capable of being developed in steels by the practice of

45 this invention, with the properties available in the same steels during various stages of the process and with other methods for processing the same steels to take the equivalent reduction at equivalent temperature, as in the elevated temperature reduction process of the aforementioned co-pending applications. In the presentation of data on steels reduced at elevated temperature, the values set forth are arbitrarily selected to represent the better of the values for the respective properties in steels processed within the described temperature range. For example, the better tensile strength and yield strength properties will be found in steels drawn at a temperature within the range of about 400°-900° F. while the better values of elongation and reduction in area will be found in the steels drawn at a temperature within the upper portion of the elevated temperature reduction range.

50 60 In the tables, the following abbreviations have been used:

(A)=air-cooled after drawn.

(Q)=quenched in oil or water after drawn.

ETD=drawn at elevated temperature.

55 AQT<sub>900</sub>=austenitized and quenched steel which has been tempered at 900° F.

AQT<sub>400</sub>=austenitized and quenched steel which has been tempered at 400° F.

65 70 AQT<sub>900CD</sub>=austenitized and quenched steel which has been tempered at 900° F. and drawn at ambient temperature.

AQT<sub>900D</sub>=austenitized and quenched steel which has been tempered at 900° F. and drawn at elevated temperature.

75

**Table XII**  
[C-1018 Steel.]

| Process                               | Total Red., Percent | Tensile Strength, p.s.i. | Yield Strength, p.s.i. | Elongation, 1/4", Percent | Red. of Area, Percent | Warpage Factor Range | Izod Impact, 70° F., Ft. Lbs. | Pull Range, Lbs. | Hardness, DPN, MR |
|---------------------------------------|---------------------|--------------------------|------------------------|---------------------------|-----------------------|----------------------|-------------------------------|------------------|-------------------|
| Hot Roll                              |                     | 68,375                   | 46,875                 | 36.0                      | 67.9                  | +.021                | 87.0                          |                  | 151               |
| Cold Drawn (A)                        | 17.2                | 103,000                  | 103,000                | 13.0                      | 52.1                  | -.003                | 23.0                          | 11,450           | 223               |
| ETD (A)                               | 17.2                | 116,250(a)               | 116,250(a)             | 27.5(b)                   | 58.8(b)               | -.001--.184          | 11.7(c)                       | 10,305-8,588     | 266               |
| H.R. Quenched and Tempered at 900° F. |                     | 90,750                   | 72,000                 | 25.5                      | 31.7                  | -.069                | (72.7)                        |                  | 213               |
| AQT <sub>900</sub> CD (A)             | 17.2                | 117,750                  | 117,500                | 11.5                      | 60.7                  | -.058                | (46.0)                        | 14,885           | 262               |
| AQT <sub>900</sub> D (A)              | 17.2                | 128,750(d)               | 128,750(d)             | 24.0(e)                   | 69.2(e)               | +.190-0              | 25.0(f)                       | 13,168-11,450    | 303               |
| H.R. Quenched and Tempered at 400° F. |                     | 109,750                  | 75,000                 | 19.5                      | 55.6                  | -.240                | 43.0                          |                  | 285               |
| AQT <sub>400</sub> CD (A)             | 17.2                | 138,000                  | 137,500                | 9.5                       | 42.8                  | +.040                | 8.7                           | 18,465           | 343               |
| AQT <sub>400</sub> D (A)              | 17.2                | 147,500(j)               | 147,500(j)             | 17.5(e)                   | 68.3(e)               | +.052--.110          | 8.7(h)                        | 15,288-9,733     | 366               |

(a)=at 540° F. (e)=at 900° F.  
(b)=at 1,000° F. (f)=at 380° F.  
(c)=at 450° F. (g)=at 585° F.  
(d)=at 550° F. (h)=at 230° F.

**Table XIII**

[C-1144 Steel.]

| Process                                 | Total Red., Percent | Tensile Strength, p.s.i. | Yield Strength, p.s.i. | Elongation, 1/4", Percent | Red. of Area, Percent | Warpage Factor Range | Izod Impact, 70° F., Ft.-Lbs. | Hardness, DPN, MR |
|-----------------------------------------|---------------------|--------------------------|------------------------|---------------------------|-----------------------|----------------------|-------------------------------|-------------------|
| Hot Roll                                |                     | 108,000                  | 70,500                 | 23.0                      | 46.1                  | +.004                | 32.7                          | 220               |
| Cold Drawn (A)                          | 21.6                | 132,750                  | 118,750                | 13.0                      | 34.4                  | +.732                | 18.0                          | 266               |
| ETD (A)                                 | 21.6                | 150,250(a)               | 145,000(a)             | 15.0(b)                   | 42.3(b)               | +.711-+.170          | 35.3(b)                       | 318               |
| H.R. Quenched and Tempered at 1,100° F. |                     | 126,250                  | 115,500                | 20.0                      | 54.4                  | +.046                | 35.7                          | 285               |
| AQT <sub>1100</sub> CD (A)              | 21.6                | 145,250                  | 125,500                | 10.0                      | 36.2                  | +.888                | 35.3                          | 291               |
| AQT <sub>1100</sub> D (A)               | 21.6                | 162,750(c)               | 162,750(c)             | 22.0(d)                   | 54.4(d)               | +.810-+.043          | 52.7(d)                       | 336               |
| H.R. Quenched and Tempered at 900° F.   |                     | 166,500                  | 156,000                | 14.5                      | 46.5                  | +.014                | 25.0                          | 371               |
| AQT <sub>900</sub> CD (A)               | 21.6                | 181,750                  | 180,000                | 11.5                      | 42.3                  | +.1.252              | 51.5                          | 350               |
| AQT <sub>900</sub> D (A)                | 21.6                | 213,750(e)               | 212,500(e)             | 15.0(f)                   | 43.2(f)               | +.1.230-+.142        | 50.0(g)                       | 402               |

(a)=at 660° F. (e)=at 610° F.  
(b)=at 940° F. (f)=at 880° F.  
(c)=at 630° F. (g)=at 350° F.  
(d)=at 955° F.

**Table XIV**

[C-1080 Steel.]

| Process                                 | Total Red., Percent | Tensile Strength, p.s.i. | Yield Strength, p.s.i. | Elongation, 1/4", Percent | Red. of Area, Percent | Warpage Factor Range | Izod Impact, 70° F., Ft.-Lbs. | Hardness, DPN, MR |
|-----------------------------------------|---------------------|--------------------------|------------------------|---------------------------|-----------------------|----------------------|-------------------------------|-------------------|
| Hot Roll                                |                     | 144,500                  | 76,000                 | 12.5                      | 17.0                  | +.025                | 4.7                           | 296               |
| Cold Drawn (A)                          | 15.7                | 170,500                  | 148,500                | 5.0                       | 14.5                  | +.077                | 3.3                           | 324               |
| ETD (A)                                 | 15.7                | 189,000(a)               | 186,000(a)             | 10.0(b)                   | 12.4(b)               | +.077--.038          | 5.0(c)                        | 378               |
| H.R. Quenched and Tempered at 1,200° F. |                     | 133,500                  | 103,000                | 21.0                      | 41.9                  | -.002                | 34.7                          | 276               |
| AQT <sub>1200</sub> CD (A)              | 15.7                | 154,250                  | 133,000                | 12.5                      | 43.2                  | +.039                | 20.0                          | 324               |
| AQT <sub>1200</sub> D (A)               | 15.7                | 170,250(d)               | 170,000(d)             | 20.0(e)                   | 38.9(e)               | +.101-+.023          | 38.7(e)                       | 318               |
| H.R. Quenched and Tempered at 700° F.   |                     | 256,000                  | 217,500                | 10.0                      | 25.1                  | +.093                | 5.3                           | 490               |
| AQT <sub>700</sub> CD (A)               | 15.7                | 261,000                  | 260,000                | 0                         | 0                     | +.140                | 4.0                           | 502               |
| AQT <sub>700</sub> D (A)                | 15.7                | 303,000(f)               | 303,000(f)             | 3.6(f)                    | 14.1(f)               | +.210-+.016          | 25.3(g)                       | 438               |

(a)=at 610° F. (e)=at 935° F.  
(b)=at 940° F. (f)=at 580° F.  
(c)=at 815° F. (g)=at 900° F.  
(d)=at 630° F.

**Table XV**

[4140 Steel.]

| Process                     | Total Red., Percent | Tensile Strength, p.s.i. | Yield Strength, p.s.i. | Elongation, 1/4", Percent | Red. of Area, Percent | Warpage Factor Range | Izod Impact, 70° F., Ft.-Lbs. | Hardness, DPN, MR |
|-----------------------------|---------------------|--------------------------|------------------------|---------------------------|-----------------------|----------------------|-------------------------------|-------------------|
| Hot Roll                    |                     | 140,000                  | 105,750                | 15.0                      | 42.8                  | -.004                | 9.0                           | 307               |
| Cold Drawn (O)              | 19.9                | 160,000                  | 153,000                | 9.0                       | 48.9                  | +.159                | 6.0                           | 330               |
| ETD (O)                     | 19.9                | 195,000(a)               | 191,250(a)             | 17.5(b)                   | 45.7(b)               | +.262-+.026          | 12.0(b)                       | 402               |
| AQT <sub>1,100</sub> CD (O) | 19.9                | 182,000                  | 172,000                | 16.0                      | 52.5                  | +.089                | (39.0)                        | 353               |
| AQT <sub>1,100</sub> D (O)  | 19.9                | 197,000(c)               | 195,500(c)             | 22.0(b)                   | 61.3(b)               | +.191-+.089          | 33.0(d)                       | 402               |
| AQT <sub>600</sub> D (O)    | 19.9                | 278,000(e)               |                        | 22.5(f)                   | 62.0(f)               | +.517-+.013          | 33.0(g)                       | 594               |

(a)=at 705° F. (e)=at 600° F.  
(b)=at 960° F. (f)=at 980° F.  
(c)=at 690° F. (g)=at 815° F.  
(d)=at 590° F.

Comparison of the data will show that austenitizing and quenching followed by reduction at elevated temperature provides improvements in properties over the same steels which have been merely subjected to an elevated temperature reduction step from the standpoint of tensile strength, yield strength, and hardness for both air cooled and quenched specimens. Ductility and impact strengths are also improved by the practice of this invention as compared to elevated temperature reduction or cold reduction without previously having effected a phase change by austenitizing and quenching. The residual stress characteristics are somewhat of the same character as are secured by elevated temperature reduction alone.

It will be apparent from the foregoing that the combination of steps embodied in the practice of this invention is capable of use to produce steels having new and improved combinations of properties and in which various of its properties, such as its strength properties, elasticity, hardness, and machinability are materially improved over values which are capable of being secured in equivalent steels by other conventional cold finishing systems which have heretofore been employed.

It will be understood that changes may be made in the details of handling and processing without departing from the spirit of the invention, especially as defined in the following claims.

1. The metallurgical process for treating steel of the non-austenitic type having a pearlitic structure in a matrix of free ferrite comprising the combination of steps of heating the steel to austenitizing temperature and quenching the steel to form martensite, tempering the steel, and advancing the tempered martensitic steel through a draw die to effect reduction in cross-sectional area in a drawing operation while the steel is at a temperature within the range of 400° F. to the lower critical temperature for the steel composition.

2. The metallurgical process for treating steel of the non-austenitic type having a pearlitic structure in a matrix of free ferrite comprising the combination of steps of heating the steel to austenitizing temperature and quenching the steel to form martensite, tempering the steel, and advancing the tempered martensitic steel through an extrusion die to effect reduction in cross-sectional area in the extrusion operation while the steel is at a temperature within the range of 400° F. to the lower critical temperature for the steel composition.

3. The metallurgical process for treating steel which strain-hardens and which hardens by some mode of precipitation when worked at a temperature between 200° F. and the lower critical temperature for the steel composition comprising the combination of steps of heating the steel to austenitizing temperature and quenching the steel to form martensite, tempering the steel by heating to a temperature below the lower critical temperature of the tempered martensitic steel composition, and advancing the steel through a die to effect reduction in cross-sectional area while the steel is at a temperature within the range of 400° F. to the lower critical temperature for the steel composition.

4. The metallurgical process for treating steel which strain-hardens and which hardens by some mode of precipitation when worked at a temperature between 200° F. and the lower critical temperature for the steel composition comprising the combination of steps of heating the steel to austenitizing temperature and quenching the steel to form martensite, tempering the steel by heating to a temperature below the lower critical temperature of the tempered martensitic steel composition, and advancing the steel through a draw die to effect reduction in cross-sectional area by a draw operation while the steel is at a temperature within the range of 400° F. to the lower critical temperature for the steel composition.

5. The metallurgical process for treating steel which strain-hardens and which hardens by some mode of precipitation when worked at a temperature between 200° F. and the lower critical temperature for the steel composition comprising the combination of steps of heating the steel to austenitizing temperature and quenching the steel to form martensite, tempering the steel by heating to a temperature below the lower critical temperature of the tempered martensitic steel composition, and advancing the steel through an extrusion die to effect reduction in cross-sectional area while the steel is at a temperature range within 400° F. to the lower critical temperature for the steel composition.

6. The metallurgical process for treating steel which strain-hardens and which hardens by some mode of precipitation when worked at a temperature between 200° F. and the lower critical temperature for the steel composition comprising the combination of steps of heating the steel to austenitizing temperature and quenching the steel to form martensite, tempering the steel by heating to a temperature below the lower critical temperature of the tempered martensitic steel composition, and rolling the steel to effect reduction in cross-sectional area by the rolling operation while the steel is at a temperature within the range of 400° F. to the lower critical temperature for the steel composition.

7. The metallurgical process for treating steel which strain-hardens and which hardens by some mode of precipitation when worked at a temperature between 200° F. and the lower critical temperature for the steel composition comprising the combination of steps of heating the steel to austenitizing temperature and quenching the steel to form martensite, tempering the steel by heating to a temperature below the lower critical temperature of the steel composition, and advancing the tempered martensitic steel through a die to effect reduction in cross-sectional area while the steel is at a temperature within the range of 400° F. to the lower critical temperature for the steel composition and air-cooling the steel after advancing through the die in the elevated-temperature-reduction step.

8. The metallurgical process for treating steel which strain-hardens and which hardens by some mode of precipitation when worked at a temperature between 200° F. and the lower critical temperature for the steel composition comprising the combination of steps of heating the steel to austenitizing temperature and quenching the steel to form martensite, tempering the steel by heating to a temperature below the lower critical temperature of the steel composition, advancing the steel through a die to effect reduction in cross-sectional area while the steel is at a temperature within the range of 400° F. to the lower critical temperature for the steel composition and quenching the steel rapidly to cool the steel after advancement through the die at elevated temperature.

9. A steel product having new and improved physical and mechanical properties produced by the method of claim 3.

#### References Cited in the file of this patent

#### UNITED STATES PATENTS

|           |         |               |
|-----------|---------|---------------|
| 1,018,369 | Potter  | Feb. 20, 1912 |
| 2,435,511 | Rice    | Feb. 3, 1948  |
| 2,448,753 | Weesner | Sept. 7, 1948 |

#### OTHER REFERENCES

Alloys of Iron and Carbon, vol. 1, Epstein, pp. 177-178, 1936.

Metal Progress, May 1945, p. 938.

Dunn: Iron & Steel Engineer, pages 51-57 and 77, July 1946.

Bullens: Steel and Its Heat Treatment, pages 311-326, 1948.